

P. F. SARRON AND J. SIMON.  
ELECTROCONVERTER FURNACE,  
APPLICATION FILED JUNE 8, 1918.

1,325,114.

Patented Dec. 16, 1919.



FIG. 3



FIG. 5

FIG. 6

Witnesses

Jean Sarron  
Charles Fire.

Inventors

Paul François Sarron  
Jules Simon

# UNITED STATES PATENT OFFICE.

PAUL FRANÇOIS SARRON AND JULES SIMON, OF LYON, FRANCE.

## ELECTROCONVERTER-FURNACE.

1,325,114.

Specification of Letters Patent. Patented Dec. 16, 1919.

Application filed June 8, 1918. Serial No. 238,899.

To all whom it may concern:

Be it known that we, PAUL FRANÇOIS SARRON and JULES SIMON, citizens of the French Republic, both of Lyon, France, have invented certain new and useful Improvements in Electroconverter - Furnaces, of which the following is a specification.

This invention relates to improvements in electro-converter furnaces and process of treatment for the manufacture of ordinary and special steels thereby.

By the invention furnaces known as "converters" can be rapidly transformed into electric furnaces, which allows the advantages peculiar to both types of apparatus to be utilized and a special operative method to be performed for the economical manufacture of the best steels, by treating more or less pure products and freeing, if necessary, the metal obtained from the greater part of the gases which are found dissolved therein.

The following description relates by way of example to an acid converter with lateral blast, transformed into an electric furnace with two electrodes.

In the annexed drawings:

Figure 1 is a vertical section through the axis 1-1 of the furnace placed in the horizontal position and arranged for working as electric furnace;

Fig. 2 is a vertical section on line 2-2 of Fig. 3;

Fig. 3 is a horizontal section on line 3-3 of Fig. 1;

Fig. 4 is a vertical section through the axis 1-1 of the furnace, but placed in an upright position and arranged for working as converter;

Fig. 5 an elevation on a smaller scale of the whole structure forming the furnace, its electrodes, the suspension cables, the cab of the regulating devices and the traveling bridge supporting this cab.

Fig. 6 is a vertical section of the insulating device for an electrode for a furnace with basic lining.

In the outer casing *a* and the lining *b* of the apparatus are provided openings which, when the apparatus works as converter, are closed by plugs *c* of a composition identical with or similar to that of the lining; the cover *d* is then open in the position illustrated in Fig. 4.

In order to transform the apparatus into an electric furnace, it is brought into the

horizontal position and the plugs are removed by means of the rings *e*; then the openings can be used for effecting the charging of the apparatus, although this can also be effected through the nozzle *f*. This done, 60 metal sleeves *g* are then inserted into the plug openings and fixed to the furnace plates by means of any suitable keying means; it is in these sleeves, which may be cooled or not by a circulation of air or 65 water, that the electrodes *h* slide, suspended by the cables *i* which may be provided with automatic regulating devices. These apparatus which raise or lower the electrodes and their electric connections are preferably arranged in a cab *j* shown in Fig. 5 supported on a traveling bridge *k* which can move above the furnace and the flue *l*. The current is conveyed to the electrodes by the flexible conductors *m*, the bars *n* and the 70 metal jaws *o* fixed closely on the electrodes by means of the bolts *p*. These jaws are guided by metal rods *q* integral with the sleeves *g* and carry at their upper part abutment screws *r*. This device secures the guiding of the electrodes when the furnace is inclined for the washings which are effected through the nozzle *f*, the tapping of the metal being preferably effected through the channel *s*, plugged normally by the refractory plug *t*. The tapping is thus effected 75 without having to incline the apparatus.

When it is desired to withdraw the electrodes from the furnace they are raised until the jaws abut against the nuts *r*; at that 80 moment the end *u* of the electrodes, which is found to be the hottest, has engaged in the socket end *v* of the sleeve *g*; the electrodes are removed from the muffles and the cables *i* continue to be pulled; the sleeves then 85 accompany the electrodes, protecting them from the action of the air, while the bridge *k* transports them over and lowers them into another furnace or into heat retaining devices comprising cylinders lined with refractory material in which they can remain until again required for use.

The general arrangement, which has just been described by way of example, can be applied to any converter other than an acid 105 converter with lateral blast; the blast can be effected through the bottom or in any manner whatever, but in all cases the air-chamber is provided with a tube *x*, with sliding-valve *y*, connected to a suction-machine 110

capable of producing a relative vacuum in the apparatus, after it has been closed as hermetically as possible by means of the plugs *c* and the lid *d*, which latter need not be integral with the apparatus and can be constructed like a digester stopper.

The lining may be neutral or basic; in the latter case the electrodes are not in direct contact with the sleeves *g*. In order to prevent the current passing into these sleeves from being diverted to the magnesian lining which becomes conductive at high temperature, a refractory packing *z* formed of a bad conductor is interposed between the electrode and the sleeve as illustrated in Fig. 6.

The furnace may be an arc furnace, with or without magnetic blast, or may have an arc and resistance combined comprising either only the top electrodes, or one or more top electrodes and one or more polar masses embedded in that part of the lining which forms the sole, or finally one or more top electrodes and a wholly or partially conductive sole. It is evident that suitable electrical insulation must correspond to each particular case; precautions are also to be taken for avoiding the closing of the magnetic circuits and to hinder the production of Foucault currents.

Further, the upper electrodes can also be suspended from posts placed beside the furnace, near the operating devices.

These electrodes can moreover be protected by the known means such as jackets of sheet-steel, facings of silicate of soda and asbestos held in place by a metal grating, etc.

The general method for the manufacture of steel, starting from any suitable materials, is as follows:

In the first place two electro-converter furnaces are disposed, one with acid lining, the other with basic lining. In the former the fusion of the material, cast-iron, filings of cast-iron or steel, dross, etc., is effected.

If the products to be melted do not contain much carbon some carbon is added to the charge in order that the melted product may form a casting; also, if necessary, the desired additions are made so that this casting contains a proportion of silicon which makes it suitable to be converted on an acid lining. When the fusion is terminated, the apparatus is brought into the converting position and the blast is operated until the

greater part of the silicon is oxidized; at this moment the bath has become very hot; the blast is stopped and the metal is run into a heated pocket which is emptied into the electro-converter basic furnace which has been previously charged with the lime required for dephosphorization; then the conversion is terminated. At the end of the superblowing the greater part of the phosphorus is burnt, but there still remains too

much of it in the metal to allow the latter to form a good steel; it is also necessary to subject it to an electric super-refining which will, besides, serve for the elimination of the sulfur. For the purpose it is washed after the superblowing and before removing the plugs *e* the lid *d* is turned down on to the nozzle. All the openings are seen to be well closed and the suction machine is started working, after having opened the valve *v*; a relative vacuum is thus created above the bath and the excess of gases dissolved in the metal is eliminated which greatly contributes to improve the final product. This being done, the electrodes are put into place, after having inserted the materials necessary for the formation of a new basic slag and the current is turned on; the amount of scale is relatively slight, because a part of the oxid of iron which has formed in the course of the super-blowing serves to oxidize the impurities left in the bath. The washing is repeated and the refining of the metal terminated in the usual manner.

This general method enables steels of superior quality to be manufactured from any products, much more quickly than in the Martin or the electric furnace; the operation is simplified if one has well defined products at disposal, if, for instance, they contain for example very little phosphorus and sulfur they can be treated solely in an acid electro-converter furnace, which effects the fusion of the materials, the conversion, the elimination of the dissolved gases and the fusion of the added matters, which last may be as considerable as desired. If the products which are to be treated contain much phosphorus they are treated only in a basic electro-converter furnace, which effects the fusion, the conversion, the elimination of the dissolved gases and the electric super-refining.

It is evident that this process applies equally well to liquid castings prepared outside the electro-converter furnace and coming from a blast-furnace, a smelting-furnace or other apparatus; these castings are treated, according to their chemical composition, either only in an acid electro-converter furnace, or only in a basic electro-converter furnace, or, by means of fractional conversion, first in an acid electro-converter furnace, then in a basic electro-converter furnace.

Finally, the electro-converter furnace may serve singly as converter or singly as electric furnace. The fusion of the metal can otherwise be non-electrically effected, for instance by means of heavy oil or of gases brought through burners introduced through the tuyers.

The advantages resulting from the use of the electro-converter furnaces and from the

operating method which they allow are as follows:

The operations of fusion, conversion and super-refining being generally effected in a single electro-converter furnace, the calorific yield is better than if these operations were effected in several apparatus. The installation is less costly and less cumbersome and the manufacture, which is easier to superintend, requires the least amount of manual labor. The construction of the furnace is simple, the up-keep easy, as the refractory lining, is easily repairable. The vault does not form a delicate part of the apparatus as in the ordinary electric furnaces.

The process of manufacture is rapid and economical, as the refining is almost wholly effected in a few minutes and without the necessity of heating the metal. The economy is also due to the fact that carbureted materials are treated which melt at a comparatively low temperature, in an apparatus which has been left by the preceding operation at a very high temperature in great part due to the exothermic reactions which have been effected during the conversion. The amount of heat to be electrically furnished is therefore relatively slight.

Further, the electro-converter furnaces can be almost hermetically closed; owing to their method of construction; it is therefore possible to create therein a relative vacuum, which enables the greater part of the gases contained in the metal to be eliminated.

What we claim as our invention and desire to secure by Letters Patent of the United States is:—

1. An electroconverter furnace comprising

ing a casing of the converter type, a cover therefor, a refractory lining for said casing, 40 said casing and lining being provided with openings, sleeves fitted in said openings, removable electrodes passing through said sleeves and slidable therein, means for conveying current to said electrodes, means for suspending and effecting the sliding movement of said electrodes and for removing them from said sleeves and plugs for closing said openings when said electrodes are removed from said sleeves.

2. An electroconverter furnace comprising a casing of the converter type, a cover therefor, a refractory lining for said casing, said casing and lining being provided with openings, sleeves fitted in said openings, 55 means for cooling said sleeves, electrodes passing through said sleeves and slidable therein, jaws fixed on said electrodes, metal rods fixed to said sleeves and passing through said jaws, bars fixed to said electrodes, flexible electric conductors attached to said bars, means for suspending and effecting the sliding movement of said electrodes and for removing them from said sleeves, and plugs for closing said openings 60 when said electrodes are removed from said sleeves.

In witness whereof we have signed this specification in the presence of two witnesses.

PAUL FRANÇOIS SARRON  
JULES SIMON.

Witnesses:

JEAN GERMAIN,  
GRADY CORBITT.